

# United States Patent [19]

Brody

[11] 4,442,266

[45] Apr. 10, 1984

[54] MELT SPINNING OF POLYPROPYLENE

[75] Inventor: Harry Brody, Harrogate, England

[73] Assignee: Imperial Chemical Industries Limited, London, England

[21] Appl. No.: 268,252

[22] Filed: May 29, 1981

[30] Foreign Application Priority Data

May 13, 1981 [GB] United Kingdom ..... 8114626

[51] Int. Cl.<sup>3</sup> ..... C08L 67/06

[52] U.S. Cl. ..... 525/173; 264/176 F; 525/174; 525/445

[58] Field of Search ..... 264/176 F; 525/445, 525/173, 174

[56] References Cited

U.S. PATENT DOCUMENTS

3,591,673 7/1971 Pollack ..... 525/425

3,884,989 5/1975 Blomberg ..... 525/425

3,935,337 1/1976 Taylor ..... 427/180

4,189,549 2/1980 Matsunaga et al. ..... 525/444

4,386,174 5/1983 Cogswell et al. ..... 525/425

FOREIGN PATENT DOCUMENTS

45-11834 4/1970 Japan ..... 525/425

45-11833 4/1970 Japan ..... 525/425

55-82150 10/1980 Japan ..... 264/176 F

2008598 6/1979 United Kingdom ..... 264/176 F

Primary Examiner—Jay H. Woo

Attorney, Agent, or Firm—Cushman, Darby & Cushman

[57] ABSTRACT

A process of melt spinning polypropylene the improvement comprising adding to the polypropylene before it is melt spun, a small proportion of a polymer capable of forming an anisotropic melt in the temperature range at which the polypropylene may be melt spun and then melt spinning the polymers together at a wind up speed of less than 1000 meters per minute whereby in the process there is a suppression of wind up speed compared with the process carried out in the absence of the added polymer.

5 Claims, 2 Drawing Figures





Fig. 1

TRUE STRESS AT  
50% STRAIN  
(cN/tex)



Fig. 2

## MELT SPINNING OF POLYPROPYLENE

This invention relates to the manufacture of fibres of polypropylene by melt spinning and drawing.

According to this invention we provide a process of melt spinning polypropylene in which there is added to the polypropylene a small proportion of a polymer capable of forming an anisotropic melt in the temperature range at which the polypropylene may be melt spun, and the polymers are then melt spun together in intimate mixture at a wind up speed of less than 1000 meters per minute whereby in the process there is a suppression of wind up speed compared with the process carried out in the absence of the added polymer.

We also provide fibres of polypropylene containing a small proportion of polymer capable of forming an anisotropic melt which have been spun at a wind up speed of less than 1000 meters per minute.

We prefer that the overlap of the anisotropic melt temperature range of the added polymer and the spinnable temperature range of the polypropylene is at least 5° C. and preferably much more and we prefer to incorporate between 0.1% and 10% by weight of the added polymer.

By "a polymer capable of forming an anisotropic melt" is meant either that the polymer forms such a melt when heated to a particular temperature range, characteristic of the polymer (this type is termed a "thermotropic" polymer) or can be induced to form such a melt by the application of shear to the melt. The latter state is characterised by the persistence of the anisotropic condition for a period of a second or two after the melt ceases to be sheared. This distinguishes it from the well-known observation that, for example, a polyethylene terephthalate melt will exhibit order when sheared by passing the melt through a tube. Such order disappears immediately the melt ceases to be sheared. Some polymers may show both thermotropic and shear-induced anisotropy. Polymers exhibiting such anisotropic melt behaviour have been called liquid crystal polymers and in what follows will be referred to as LC polymers. Polypropylene will be referred to as the host polymer. Some tests for establishing whether a polymer shows anisotropic melt behaviour have been published in British Pat. No. 1,507,207.

Many patent specifications were published during the 1970's disclosing LC polymers. In general any known LC polymer can be chosen for addition to the host polymer according to the invention provided that it can be processed in the same melt temperature range as the host polymer and provided that it does not react chemically with the host polymer to cause significant polymer degradation during melt spinning.

For use with polypropylene as the host polymer particularly suitable LC polymers are copoly chloro 1,4 phenylene ethylene dioxy 4,4' dibenzoate/terephthalate (CLOTH) and copoly ethylene terephthalate/p-oxybenzoate (designated X7G in the following examples).

The effect of LC polymers is that of WUS suppression i.e. the properties of the spun fibre are those that would be obtained from a fibre spun at lower WUS. As the WUS increases in normal spinning where LC polymers are not used certain properties of fibres increase or decrease continuously. These properties can therefore be used to measure the degree of WUS suppression. In the case of polypropylene, the property that has been

chosen has been the true stress at 50% strain derived from the Instron stress/strain curve of the spun fibre. This normally increases smoothly with WUS, so that a reduction of this stress at a given WUS is indicative of WUS suppression.

## BRIEF DESCRIPTION OF THE DRAWINGS

FIG. 1 is a graph showing plots of the specific stress (load divided by initial tex) versus strain for yarns of polypropylene blends; and

FIG. 2 is a graph showing plots of the true stress at 50% strain (specific stress multiplied by 1.5) versus wind up speed (mpm) for yarns of polypropylene blends.

This invention will now be described with reference to the following Examples:

In the experiments described below two different LC polymers were mixed with polypropylene as host polymer. The LC polymers were:

(In Example 1) Copoly chloro 1,4, phenylene ethylene dioxy 4,4' dibenzoate/terephthalate (CLOTH). This polymer was prepared according to Example 3 of U.S. Pat. No. 3,991,013. It had an inherent viscosity of 1.07 dl/g at 25° C. in a 0.5% solution of 30% trifluoracetic acid and 70% dichloromethane. The polymer melted in the range 215°/225° C. to give an anisotropic melt as observed in a Leitz hot stage fitted to a Leitz SM POL model polarising microscope. It had a melt viscosity of 50 Ns/m<sup>2</sup> at 10<sup>4</sup> N/m<sup>2</sup> and 270° C.

(In Example 2) copoly ethylene terephthalate/p-oxybenzoate (X7G). This was prepared according to W J Jackson and H F Kuhfuss, J Poly Sci, (Poly Chem Edition), 2043, 14 (1976) and U.S. Pat. Nos. 3,778,410 and 3,804,805. It had an inherent viscosity of 0.34 dl/g at 25° C. in a 1% solution of dichloroacetic acid. The polymer gave an anisotropic melt at 188° C. It had a melt viscosity of 220 Ns/m<sup>2</sup> at 10<sup>4</sup> N/m<sup>2</sup> and 270° C. The above LC polymers were blended separately in the weight concentrations mentioned below with Ultron grade polypropylene containing pro-degradant in a BETOL single screw extruder which had a 19 mm diameter 'nylon screw' of 30:1 L/D ratio. The screw feed was 100 rpm with the feed zone at 210° C. and observed barrel temperatures from feed zone to die end of 255°, 270°, 275° and 280° C. The blend leaving the die had a temperature of 260°-265° C. The lace was 2 mm diameter and water quenched, with a slight haul-off to give smooth running. It was then cut with a lace cutter.

The LC polymers were all dried overnight in a vacuum oven at 60°-70° C. before blending. The polypropylene was not predried. Mix weights of about 700 grams were fed to the extruder and about the first 200 grams dumped to clear out the previous 'tail'.

As a control, polypropylene without addition of LC polymer, was also passed through the extruder.

The blends so formed were spun on a rod spinner through 15 thou spinneret holes without quench air on a conditioner tube. Candles were made at 135° C. with 8 minutes candling time. The throughput was 27 g/hr/hole and the extrusion temperature finally selected after various trials was 288° C. Spin finish was applied in a conventional manner. The yarn was wound on a conventional wind-up unit for wind up speeds (WUS) up to 600 mpm, while a capstan was used for WUS greater than 600 mpm and the yarn rewound onto bobbins.

It was found that stress-strain curves offer a satisfactory basis for comparing products obtained from blends

of an LC polymer and polypropylene with the control. In general the stress at a given strain increases fairly uniformly and so the true stress at a fixed strain of 50% provides a good basis for evaluating the degree of wind up speed suppression.

The results obtained are tabulated in Table 1.

FIG. 1 also shows the effect of 6% by weight of CLOTH on the stress-strain curves of polypropylene. FIG. 2 further shows the effect of both 6% CLOTH and 3% X7G (both by weight) on the stress curves of polypropylene at various WUS. (In FIG. 1 it should be noted that the stress is not a true stress but is the 'specific stress', ie the load divided by the initial tex).

TABLE 1

| BLEND    | WUS<br>(mpm) | TRUE STRESS AT<br>50% STRAIN<br>(cN/TEX) | EQUIVALENT<br>LOWER WUS*<br>(mpm) |
|----------|--------------|------------------------------------------|-----------------------------------|
| CONTROL  | 200          | 4.4                                      |                                   |
|          | 300          | 6.7                                      |                                   |
|          | 400          | 8.1                                      |                                   |
|          | 500          | 8.2                                      |                                   |
|          | 600          | 10.3                                     |                                   |
|          | 1000         | 12.5                                     |                                   |
| 6% CLOTH | 200          | 3.4                                      | —                                 |
|          | 300          | 4.4                                      | 200                               |
|          | 400          | 5.7                                      | 250                               |
|          | 600          | 7.2                                      | 360                               |
|          | 1000         | 10.8                                     | 675                               |
|          |              |                                          |                                   |
| 3% X7G   | 200          | 3.8                                      |                                   |
|          | 300          | 4.5                                      | 225                               |
|          | 400          | 5.4                                      | 280                               |
|          | 500          | 8.1                                      | 350                               |
|          | 600          | 8.3                                      | 425                               |

\* Calculated from curves in FIG. 2.

The effect of the LC polymers was appreciable with 6% CLOTH producing almost a 50% fall in effective WUS.

Table 2 shows that the melt flow index (MFI) of the fibres containing an LC polymer were essentially the same as the control, within experimental error, so that

the effect is not due to the degradation of the polypropylene.

TABLE 2

|       | BLEND    | MFI | MOLECULAR<br>WEIGHT |
|-------|----------|-----|---------------------|
| CHIP  | CONTROL  | 66  | 212,000             |
|       | 6% CLOTH | 94  | 192,000             |
| FIBRE | CONTROL  | 120 | 179,000             |
|       | 3% X7G   | 184 | 159,000             |
|       | 6% CLOTH | 140 | 171,000             |

I claim:

1. A process of melt spinning polypropylene the improvement comprising adding to the polypropylene before it is melt spun, a small proportion of a polymer capable of forming an anisotropic melt in the temperature range at which the polypropylene may be melt spun and then melt spinning the polymers together at a wind up speed of less than 1000 meters per minute whereby in the process there is a suppression of wind up speed compared with the process carried out in the absence of the added polymer.

2. A process as claimed in claim 1 in which the temperature range of the added polymer and the spinnable temperature range of the polypropylene is at least 5° C.

3. A process as claimed in either claim 1 or claim 2 in which between 0.1% and 10% by weight of the added polymer is added to the polypropylene.

4. A process as claimed in claim 1 in which the added polymer is either copoly chloro 1,4 phenylene ethylene dioxy 4,4' dibenzoate/terephthalate or copoly ethylene terephthalate/p-oxybenzoate.

5. Fibres of polypropylene containing a small proportion of a polymer capable of forming an anisotropic melt which have been spun at a wind up speed of less than 1000 meters per minute.

\* \* \* \* \*

40

45

50

55

60

65